

Jan. 19, 1926.

1,570,078

E. C. PITMAN

NONSTATIC PHOTOGRAPHIC FILM

Filed Sept. 16, 1920



E. C. Pitman, Inventor

By his attorney H. R. Squair.

## UNITED STATES PATENT OFFICE.

EARLE C. PITMAN, OF PARLIN, NEW JERSEY, ASSIGNOR TO E. I. DU PONT DE NEMOURS & COMPANY, OF WILMINGTON, DELAWARE, A CORPORATION OF DELAWARE.

## NONSTATIC PHOTOGRAPHIC FILM.

Application filed September 16, 1920. Serial No. 410,748.

To all whom it may concern:

Be it known that I, EARLE C. PITMAN, a citizen of the United States, and a resident of Parlin, in the county of Middlesex and 5 State of New Jersey, have invented a certain new and useful Nonstatic Photographic Film, of which the following is a specification.

This invention relates to photographic 10 films having provisions for the elimination of discharges of static electricity. With the ordinary film these discharges occur when the film is stripped from the casting surface, when it is run rapidly through a cinematographic camera and under various 15 other circumstances. Such discharges cause markings on the sensitized emulsion by premature exposure thereof. It is an object of the invention to provide a film which, 20 for practical purposes of manufacture and use, will be free from static electricity, and it is also an object to improve generally upon films of the character indicated.

For convenience and brevity of description 25 I use the term "film" to denote the entire article, whether or not the article includes a sensitized emulsion; the term "film body" to denote the entire emulsion support whether or not that support is composed of 30 a plurality of layers, sub-films or pellicles; the term "backing" to denote a layer of a composite film body, which lies adjacent the other side of the film body from the side intended to directly carry the emulsion; 35 and I use the term "base" to denote the portion of a composite film body which is intended to carry the backing at one side and the emulsion at the other and to form or include the principle strength-giving portion 40 of the film. On occasion, as will appear from the context, I use the term "base" (or pellicle base) to also indicate the substance, as cellulose acetate or cellulose nitrate, which is the primary substance used to form a pellicle. 45

In the accompanying drawing I have, without restricting my invention thereto, shown a film embodying my invention, the

view being a conventional, exaggerated, cross-sectional showing.

According to my invention, I use in the film body a substance, or substances, which will make the body, either as a whole, or at its backing where one is used, more electrically conductive than is the ordinary film. In this way, I provide that such static charges as tend to be generated shall leak away, be neutralized, or be evenly distributed, before they can accumulate in such a way, or to such amount, as to be liable to 60 harmful discharge.

Thus, I may incorporate in the body a "film former" such as saponin, alkali salts of unsaturated fatty acids (such as sodium sulphorcinoleate), alkali salts of egg albumin, or alkali salts of aromatic sulphonic acids, using the film forming substance either alone or in combination with a hygroscopic substance such as glycerine, the substances selected for any specified case to be 70 soluble in the particular solvent mixture used for making the pellicle in which the substances are to be incorporated, and such as not to cause precipitation of the pellicle base used for the pellicle. The "film former" 75 acts to convert the isolated drops of moisture, collecting on the film, into a homogeneous film; thereby increasing conductivity. To the best of my knowledge the substances I call "film formers", and exemplified by the 80 substances named above, function by virtue of their common characteristics of having the ability to reduce surface tension. Therefore, lacking a common generic term for such substances, I, for convenience in claiming, 85 make reference in the claims to this ability. It is to be understood, however, that the reference is for convenience, and not by way of limitation, the intent being to include substances, exemplified by saponin and the like, which have the ability to convert isolated drops of moisture into a homogeneous film, i. e. are "film formers", regardless 90 of the particular property which enables them to so function and even though it 95 ultimately appears that that property is

other than the ability to reduce surface tension. The hygroscopic substance is advantageous in that it increases conductivity by increasing the moisture content; the "film former" is, of course, valuable whether or not the hygroscopic substance is used also, as some moisture is present in any case.

- In general, and as previously indicated, a film body, i. e. the entire emulsion support, 10 may consist of one layer only; or may consist of a plurality of layers, one of the layers being the backing, and the remainder of the body being the base or principal strength-giving layer or layers of the film body. 15 When incorporating the various substances, e. g. saponin and glycerine, in accordance with the invention, they may be placed in a film body not comprising a backing and made from any desired pellicle base, e. g. cellulose acetate; or such substances may be, in the first instance, placed in a backing and such backing applied to any desired base layer. The backing may be one which primarily functions merely by virtue of the 20 substances and, so, may not contain a pellicle base, e. g. cellulose acetate; or it may contain a pellicle base of any suitable character and either having substantially the same conductivity as the pellicle base used in making 25 the base of the film, or having a conductivity somewhat greater than that of the pellicle base used in making the base of the film and enabling the pellicle base of the backing to itself serve in giving the backing 30 a superior conductivity.

As to the use for the backing of a pellicle base which is itself of superior conductivity, I may apply a backing layer of carbohydrate ester of relatively low esterification, as 35 regards conductivity (the conductivity, and the hygroscopicity, increasing as the esterification decreases) e. g. cellulose acetate having 55% or less of combined acetic acid, that is, not over 55% of combined 40 acetic acid, and preferably having about 54%, to a film base of carbohydrate ester of relatively high esterification, as regards conductivity (the conductivity, and the hygroscopicity, decreasing as the esterification increases), e. g. cellulose nitrate having a nitrogen content of more than 11½%, preferably about 11.8%, to 12%. Experience has shown that, if proper strength is to be secured in a film primarily of cellulose nitrate, 45 then a cellulose nitrate having a nitrogen content of more than 11½% is a practical necessity despite the fact, that, used alone, it is liable to static discharges due to its non-conductivity. By the present arrangement 50 I provide a primarily cellulose nitrate film which has the strength demanded by the trade and yet is conductive and substantially non-static. As will be understood, a film of the character just indicated may, if desired, contain no added hygroscopic or film-

forming substances and yet present the advantage of conductivity to a marked degree. In such cases any suitable formulas for the base and the backing solution may be used; conveniently the below-given formulas 70 "1", and "2" with the saponin omitted, may be used for the base and the backing, respectively.

| (1)                          | Parts by weight   |           | 75 |
|------------------------------|-------------------|-----------|----|
|                              | Approximate range | Preferred |    |
| Cellulose nitrate (dry)..... | 25 to 50          | 35        | 80 |
| Camphor.....                 | 2 to 6            | 4         |    |
| Wood alcohol.....            | 90 to 150         | 120       |    |
| Acetone.....                 | 10 to 50          | 20        |    |
| Fusel oil.....               | 20 to 50          | 40        |    |
| Amyl acetate.....            | 10 to 30          | 20        |    |

While the mentioned backing is highly advantageous of itself, I have found, as previously indicated, that the incorporation, in such a backing, of conductivity-increasing substances, as a film former, alone or in combination with a hygroscopic substance, gives a particularly satisfactory film.

The mechanical operations of making films in accordance with my invention will be evident to those skilled in the art, the casting of films, and similar operations, as such, being of course well known in the art. The backing solution may be applied, and the solvents evaporated, to give the backing, in any convenient manner. Below I give formulas illustrative of films embodying my invention, it being understood that I do not restrict my invention to the examples given. In the formulas figures refer to parts by weight.

(2) For a backing containing a film former, saponin, the following formula may be used:

|                              | Approximate range | Preferred | 110 |
|------------------------------|-------------------|-----------|-----|
| Cellulose acetate (dry)..... | 4 to 16           | 6         |     |
| Saponin.....                 | 0.005 to 0.2      | 0.02      |     |
| Acetone.....                 | 100 to 140        | 120       |     |
| Wood alcohol.....            | 60 to 100         | 80        |     |

In making up, to the combined solvents add (a) the saponin and (b) the cellulose acetate, in order.

(3) For a backing containing a film former, saponin, and a hygroscopic substance, glycerine, the formula, as to ingredients, ranges, and preferred amounts, may be the same as for "2" except that it should in addition include approximately 0.25 to 15 parts, preferably 1 part, of glycerine. When preparing, add (a) the glycerine, (b) the saponin, and (c) the cellulose acetate, in order, to the combined solvents. As indicated previously, and as specifically here exemplified by the glycerine, the hygroscopic substance is 130

soluble in the particular solvent mixture used for making the pellicle, and such as not to cause precipitation of the pellicle base.

While the above backings may be of any desired thickness serving the ends sought, I have found a relatively thin backing desirable. A film base for them may be according to formula "1".

In the above backing formulas the cellulose acetate may have 55% or less of combined acetic acid or may have more than 55% combined acetic acid, but, as explained above, it is desirable that cellulose acetate having 55% or less combined acetic acid, that is not over 55% combined acetic acid, be used for the backings and that such backings be applied to a film base of cellulose nitrate having a nitrogen content of over 11½%.

To provide backings which are soluble in water and can be totally removed, say in development (after which there is no longer any danger from "static marks"), saponin and glycerine in the preferred amounts and ranges given in formulas "2" and "3" may be dissolved in 100 to 400, preferably 200, parts of denatured alcohol.

Although for purposes of specific illustration, I have made more particular reference to cellulose acetate as the pellicle base to be used for the backing, it is to be understood that I do not restrict my invention to the use of cellulose acetate as various other materials, more particularly, other carbohydrate esters, can be used for the pellicle containing the film former, alone or in combination with a hygroscopic substance.

As previously stated, the conductivity-increasing substance may be incorporated in a film body not having a backing. For example, they may be incorporated in a pellicle of cellulose nitrate, preferably having over 11½% nitrogen content. Thus:

(4) For a pellicle containing a film former, saponin, the formula as to ingredients, ranges and preferred amounts, may be the same as "1" except that it should in addition include 0.0125 to 0.3, preferably 0.05 part of saponin. In preparing, add (a) the saponin and (b) the cellulose nitrate in order to the combined solvents; and

(5) For a pellicle containing a film former, saponin, and an hygroscopic substance, glycerine, formula "4" may be used, using in addition 0.5 to 10, preferably 2, parts of glycerine. To prepare, add (a) the glycerine, (b) the saponin, and (c) the cellulose nitrate in order, to the combined solvents.

While, in describing my invention, I have referred to it as embodied in a "body without a backing" and as embodied in a "backing" it is to be understood that by neither of these terms do I exclude films wherein

the invention may have applied to its (normally) exposed surface a coating of such character as not to destroy the efficacy of the pellicle, the pellicle, from the standpoint of the present invention, yet being "without a backing" or being a "backing" as the case may be.

Although I have referred more particularly to a cellulose acetate backing on a cellulose nitrate base, it is to be understood that I may if desired apply a backing of cellulose nitrate of relatively low esterification, as regards conductivity, e. g. cellulose nitrate having a nitrogen content of not over 11½%, that is 11½% or less and preferably 10.9%, and containing or not containing added conductivity-increasing substances, to a base of cellulose acetate of relatively high esterification, as regards conductivity, e. g. cellulose acetate of more than 55% combined acetic acid, and thereby obtain, in a primarily cellulose acetate film, the combination of proper strength, and a conductivity superior to that of the film base. I have found that, as previously mentioned, cellulose nitrate, and cellulose acetate, decrease in conductivity and in hygroscopicity as the nitrogen contents, or combined acetic acid, increases, though they increase in strength, cellulose nitrate having about 11½% nitrogen content and cellulose acetate having about 55% combined acetic acid being closely comparable as regards strength, conductivity and hygroscopicity.

Of course, should it be desired for any reason, both the film base and the backing of a backed film may contain the conductivity-increasing substances.

I claim:

1. A photographic film containing a substance capable of reducing surface tension. 105

2. A photographic film containing saponin.

3. A photographic film containing a non-precipitating hygroscopic substance and a substance capable of reducing surface tension. 110

4. A photographic film containing glycerine and a substance capable of reducing surface tension. 115

5. A photographic film containing a non-precipitating hygroscopic substance and saponin.

6. A photographic film containing glycerine and saponin. 120

7. A photographic film having a base and a backing, said backing comprising 4 to 16 parts of a pellicle base and 0.005 to 0.2 parts of saponin.

8. A photographic film having a base and a backing, said backing comprising 6 parts of a pellicle base and 0.02 part of saponin. 125

9. A photographic film having a base and a backing, said backing comprising 4 to 16 parts of a pellicle base and 0.02 part of saponin. 130

parts of a pellicle base, a non-precipitating hygroscopic substance, and 0.005 to 0.2 part of saponin.

10. A photographic film having a base 6 and a backing, said backing comprising 6 parts of a pellicle base, a non-precipitating hygroscopic substance, and 0.02 part of saponin.

11. A photographic film having a base 10 and a backing, said backing comprising 4 to 16 parts of a pellicle base, 0.25 to 15 parts of glycerine, and a substance capable of reducing surface tension.

12. A photographic film having a base 15 and a backing, said backing comprising 6 parts of a pellicle base, 1 part of glycerine, and a substance capable of reducing surface tension.

13. A photographic film having a base 20 and a backing, said backing comprising 4 to 16 parts of a pellicle base, 0.25 to 15 parts of glycerine, and 0.005 to 0.2 part of saponin.

14. A photographic film having a base 25 and a backing, said backing comprising 6 parts of a pellicle base, 1 part of glycerine, and 0.02 part of saponin.

15. A photographic film having a base of cellulose ester and a backing of a different 30 cellulose ester than that of the base, the ester of said backing being of greater conductivity than that of the base.

16. A photographic film having a base of cellulose ester and a backing of a different 35 cellulose ester than that of the base, the ester of said backing being of greater hygroscopicity than that of the base.

17. A photographic film having a base of cellulose ester, and a backing of a different 40 cellulose ester than that of the base, the esterification of said backing being relatively lower, as regards conductivity, than the esterification of said base.

18. A photographic film having a base 45 element and a backing element, one of said elements being of cellulose nitrate and the other of cellulose acetate, the cellulose ester of said backing element being of greater conductivity than that of said base element.

50 19. A photographic film having a base of cellulose nitrate and a backing of cellulose acetate, the cellulose acetate of said backing being of greater conductivity than the cellulose nitrate of said base.

55 20. A photographic film having a base of cellulose nitrate and a backing of cellulose acetate, the cellulose acetate having not over 55% combined acetic acid.

60 21. A photographic film having a base of cellulose nitrate and a backing of cellulose acetate, the cellulose nitrate having a nitrogen content of over 11½% and the cellulose acetate having not over 55% combined acetic acid.

22. A photographic film having a base of 65 cellulose ester and a backing of a different cellulose ester than that of the base, the ester of said backing being of greater conductivity than that of the base, and said backing containing a conductivity-increasing 70 substance.

23. A photographic film having a base of cellulose nitrate and a backing of cellulose acetate, the cellulose nitrate having a nitrogen content of over 11½% and the cellulose 75 acetate having not over 55% combined acetic acid, and said backing containing 4 to 16 parts of cellulose acetate, and 0.005 to 0.2 part of saponin.

24. A photographic film having a base of 80 cellulose nitrate and a backing of cellulose acetate, the cellulose nitrate having a nitrogen content of over 11½% and the cellulose acetate having not over 55% combined acetic acid, and said backing containing 6 parts 85 of cellulose acetate, and 0.02 part of saponin.

25. A photographic film having a base of cellulose nitrate and a backing of cellulose acetate, the cellulose nitrate having a nitrogen content of over 11½% and the cellulose 90 acetate having not over 55% combined acetic acid, and said backing containing 4 to 16 parts of cellulose acetate, a non-precipitating 95 hygroscopic substance, and 0.005 to 0.2 part of saponin.

26. A photographic film having a base of cellulose nitrate and a backing of cellulose acetate, the cellulose nitrate having a nitrogen content of over 11½% and the cellulose acetate having not over 55% combined 100 acetic acid, and said backing containing 6 parts of cellulose acetate, a non-precipitating hygroscopic substance, and 0.02 part of saponin.

27. A photographic film having a base of 105 cellulose nitrate and a backing of cellulose acetate, the cellulose nitrate having a nitrogen content of over 11½% and the cellulose acetate having not over 55% combined acetic acid, and said backing containing 4 110 to 16 parts of cellulose acetate, 0.25 to 15 parts of glycerine, and a substance capable of reducing surface tension.

28. A photographic film having a base of cellulose nitrate and a backing of cellulose acetate, the cellulose nitrate having a nitrogen content of over 11½% and the cellulose acetate having not over 55% combined acetic acid, and said backing containing 6 parts of cellulose acetate, 1 part of 120 glycerine, and a substance capable of reducing surface tension.

29. A photographic film having a base of cellulose nitrate and a backing of cellulose acetate, the cellulose nitrate having a nitrogen content of over 11½% and the cellulose acetate having not over 55% combined acetic acid, and said backing containing 4 to 16

parts of cellulose acetate, 0.25 to 15 parts of glycerine, and 0.005 to 0.2 part of saponin. 30. A photographic film having a base of cellulose nitrate and a backing of cellulose acetate, the cellulose nitrate having a nitrogen content of over 11½% and the cellulose acetate having not over 55% combined acetic acid, and said backing containing 6 parts of cellulose acetate, 1 part of glycerine, and 0.02 part of saponin. 10 In testimony whereof I affix my signature.

EARLE C. PITMAN.